

# United States Patent [19]

Cook

[11] Patent Number: **4,601,831**

[45] Date of Patent: **Jul. 22, 1986**

[54] **ANTIMICROBIAL ADJUSTMENT  
TECHNIQUE**

[75] Inventor: **Michael M. Cook, Boxford, Mass.**

[73] Assignee: **Morton Thiokol, Inc., Chicago, Ill.**

[21] Appl. No.: **657,116**

[22] Filed: **Oct. 3, 1984**

[51] Int. Cl.<sup>4</sup> ..... **B01D 15/00**

[52] U.S. Cl. ..... **210/692; 68/18 R;  
210/764; 210/167; 210/501; 428/395**

[58] Field of Search ..... **210/688, 692, 764, 167,  
210/195.1, 196, 257.1, 284, 314, 317, 340, 341,  
343, 501; 424/16, 27, 135; 428/395; 68/18 R, 18  
F**

[56] **References Cited**

**U.S. PATENT DOCUMENTS**

- 1,575,907 3/1926 Genter ..... 210/343  
2,302,552 11/1942 Johnson ..... 210/317  
3,085,416 4/1963 D'Hooge ..... 68/18 F  
3,161,622 12/1964 Harrington et al. ..... 424/27  
3,327,859 6/1967 Pall ..... 210/266  
3,345,341 10/1967 Berry et al. ..... 424/27  
3,597,351 8/1971 Landenburg et al. ..... 210/673  
3,701,625 10/1972 Sieber ..... 8/158

- 3,715,339 2/1973 Rainer ..... 210/688  
3,829,380 8/1974 Oohara ..... 210/909  
3,959,556 5/1976 Morrison ..... 428/365  
3,979,292 9/1976 Kuhn ..... 210/120  
4,079,001 3/1978 Haase et al. ..... 210/502  
4,238,328 12/1980 Bowes et al. ..... 210/688  
4,256,588 3/1981 Hoehn et al. ..... 210/692  
4,478,714 10/1984 Blake et al. ..... 210/340  
4,483,771 11/1984 Koch ..... 210/501

**FOREIGN PATENT DOCUMENTS**

- 2355893 5/1974 Fed. Rep. of Germany ..... 210/501  
49-41270 11/1974 Japan ..... 210/688  
0686992 9/1979 U.S.S.R. ..... 210/764

*Primary Examiner*—Peter Hruskoci  
*Attorney, Agent, or Firm*—Gerald K. White

[57]

**ABSTRACT**

A system containing beds of polymeric material containing antimicrobial agents are used to adjust the antimicrobial agent concentration of treatment streams used for treating fibers with antimicrobial agents. The adjustment step is performed by passing the stream through a bed which contains the agent in a concentration different than that of the stream.

**9 Claims, 3 Drawing Figures**





Fig. 1



Fig. 2



Fig. 3

## ANTIMICROBIAL ADJUSTMENT TECHNIQUE

## CROSS REFERENCE TO OTHER APPLICATIONS

This application is related in subject matter to four other applications that were filed concurrently with this application and were commonly assigned. They are: application Ser. No. 657,119, invented by Lawrence J. Guilbault, Thomas C. McEntee, and Judith L. Koob and entitled "METHOD FOR CONTROLLING ANTIMICROBIAL CONTENT OF FIBERS"; application Ser. No. 657,118, invented by Lawrence J. Guilbault and Thomas C. McEntee and entitled "METHOD OF REMOVING A TOXICANT FROM WASTEWATER"; application Ser. No. 657,117, invented by Thomas C. McEntee, Lawrence J. Guilbault, Judith L. Koob and James F. Brophy and entitled "METHOD FOR INCORPORATING ANTIMICROBIALS INTO FIBERS"; and application Ser. No. 657,278, invented by Thomas C. McEntee, Lawrence J. Guilbault, Judith L. Koob and James F. Brophy and entitled "METHOD FOR INCORPORATING ANTIMICROBIALS INTO FIBERS".

## BACKGROUND OF THE INVENTION

This invention generally pertains to the use of polyamide beds which contain an antimicrobial agent. The beds are used to adjust the antimicrobial agent content of aqueous media. The beds are employed in combination with a system or technique which serves to perform the desired adjustment in antimicrobial agent concentration. Nylon is a typical polyamide material and 10,10'-oxybisphenoxarsine (OBPA) is a typical antimicrobial agent.

Four concurrently filed patent applications of the assignee of this invention mentioned above involve the discovery that a chemical equilibrium of antimicrobial agents exist between fibers and aqueous media containing such agent. Application Ser. No 657,119 involves a method for controlling the antimicrobial agent content of fibers during processing subsequent to the incorporation of the agent into molten material prior to the spinning step. Application Ser. Nos. 657,117 and 657,278 deal with a method for incorporating antimicrobial agents into fibers during process steps following the spinning operations. Application Ser. No. 657,118 discloses a method of removing antimicrobial agents from aqueous media. As will be observed, this application is directed to an overall system that will enable one to advantageously practice the above discussed inventions.

## SUMMARY OF THE INVENTION

The invention generally pertains to a method and system for adjusting the antimicrobial agent concentration of aqueous media. The technique comprises passing a stream which contains an antimicrobial agent through and in contact with a bed of solid polyamide material which contains a different concentration of the agent than that of the stream. Such procedure causes the antimicrobial agent to be adjusted; i.e.; either to increase or decrease, depending upon the relative concentrations.

A system for practice of the method may comprise a fiber treating vessel, reversible means for transferring antimicrobial agent containing aqueous media to and from the vessel with at least two vessels which contain

beds of polyamide materials which contains an antimicrobial agent.

## BRIEF DESCRIPTION OF THE DRAWING

5 The FIG. 1 is a schematic illustration of a system or combination of apparatus that is suitable for conducting the process of the inventions.

10 FIG. 2 is a plot illustrating OBPA uptake into a fiber and into an aqueous media as a function of contact time.

15 FIG. 3 is a plot of bath concentrations as a function of contact time.

## DETAILED DESCRIPTION OF THE INVENTION

15 It has been discovered that the concentration of antimicrobial agents in aqueous media can be substantially adjusted by contacting aqueous media with a solid polyamide material in the form of pellets, fibers, foams, granules, film or coatings. Antimicrobial agents exhibit 20 a high affinity toward polyamide materials, relative to the aqueous phase. Partition coefficients, i.e., the ratio of antimicrobial agent absorbed by the polyamide absorbant relative to that retained in the aqueous phase, at equilibrium, can be very high, ranging from 10:1 to 100:1 or higher. These favorable partition coefficients enable substantial removal of antimicrobial agents from aqueous media simply by contacting and thereby equilibrating the aqueous media with the polyamide material to facilitate rapid absorption of the antimicrobial agent by the polyamide material or, if desired, transfer of the antimicrobial agent from the polyamide material into the aqueous media. Adjustment of antimicrobial agent concentration may be effected in both directions 25 depending upon the relative concentrations in the polyamide material and in the aqueous media, contact time, face velocity, and temperature in the bed.

30 While not desiring to be bound by the following explanation, it is believed that the beneficial effects of polyamide material in adjusting the concentration of antimicrobial agents in aqueous media is due to the following. First, the agents, being somewhat polar yet decidedly organic in nature appear to have a solubility preference for polyamide relative to water. The generally low water solubility of many antimicrobial agents tends to support this preference. Secondly, polyamides in general, and nylon in particular are well known to absorb appreciable quantities of water under equilibrium conditions, up to 10-15% by weight in some instances. Thus the preference of the agent for polyamide over water and the ease by which water is absorbed into polyamide provides a driving force and transport mechanism by which agents are absorbed from aqueous media into polyamide materials.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795

The invention described in application Ser. No. 657,119 pertains to a technique for controlling the concentration of previously incorporated antimicrobial agents during processing of the fiber in aqueous media following the initial incorporation step. This technique serves to increase, decrease, or maintain essentially constant the antimicrobial agent concentration of a fiber. An important aspect of such control process is the antimicrobial agent concentration in the aqueous medium.

Fibers, articles constructed of fibers, and nonwoven fabrics are suitable for use in connection with the inventions of the above mentioned concurrently filed applications described above and include synthetic, semisynthetic, or natural fibers or blends thereof. It is expected that these methods of biocide incorporation or control would also be useful with other biocides with similar hydrophobic/solubility properties and in treating other fiber compositions such as acrylics and polyesters. Synthetic fibers include but are not limited to polyamides such as Nylon 6 and Nylon 66, polyesters, polyacrylics, and modified cellulosics.

The concept of this disclosure involves a practical method for addition and/or removal of such antimicrobial agents to or from solvents or solvent treatment baths to practice one or more of the above mentioned concurrently filed methods. This involves two or more beds of nylon resin at least one of which would contain high levels of the antimicrobial agent in the resin ("AM Rich Bed") and at least another of which would contain zero or low levels of the antimicrobial agent ("AM Poor Bed").

The antimicrobial agent may be added to the solvent used in the fiber treatment bath by passing the solvent through the AM Rich Bed at suitable combinations of face velocity, contact time and temperature until sufficient concentration of antimicrobial agent is dissolved in the solvent. Continuous cycling of the solvent through the AM Rich Bed will maintain this concentration to the bath during use. Operating parameters such as solvent temperature, bed contact time and face velocity through the bed, are readily determined by those skilled in the art and would be readily utilized to design the bed size and configuration.

The antimicrobial agent may be removed from solution by passing the solution through the "AM Poor Bed" at appropriate operating conditions to transfer all or a desired level of antimicrobial agent into the resin.

It is conceivable that when the "AM Rich Bed" is depleted of antimicrobial agent, it may be utilized as the "AM Poor Bed". A similar change may be accomplished for the AM Poor Bed as it becomes more concentrated in antimicrobial agent.

Specific antimicrobial agents that may be adjusted in concentration from aqueous media include but are not limited to those described below.

Examples of the types of microbiocidal compounds which may be employed in this invention include, but are not limited to, phenoxyarsines (including bisphenoxyarsines), phenarsazines (including bisphenarsazines), maleimides, isoindole dicarboximides, having a sulfur atom bonded to the nitrogen atom of the dicarboximide group, halogenated aryl alkanols and isothiazolinone compounds. Organotin compounds are also specifically contemplated.

The microbiocidal phenoxyarsine and phenarsazine compounds useful in the compositions of this invention include compounds represented by the formulas:



Where x is halogen or thiocyanate, y is oxygen or sulfur, z is oxygen or nitrogen, R is halo or lower alkyl, and n is 0 to 3.

Examples of these phenoxyarsines and phenarsazines include, but are not limited to, 10-chlorophenoxyarsine; 10-iodophenoxyarsine; 10-bromophenoxyarsine; 4-methyl-10-chlorophenoxyarsine; 2-tert-butyl-10-chlorophenoxyarsine; 2-methyl-8, 10-dichlorophenoxyarsine; 1, 3, 10-trichlorophenoxyarsine; 2, 6, 10-trichlorophenoxyarsine; 1, 2, 4, 10-tetrachlorophenoxyarsine; 10, 10'-oxybisphenoxyarsine (OBPA); 10-thiocyanato phenoxyarsine; and 10, 10'-thiobisphenoxyarsine; 10, 10'-oxybisphenarsazine and 10, 10'-thiobisphenarsazine.

The microbiocidal maleimide compounds useful in the compositions of this invention are exemplified by a preferred maleimide, N-(2-methylnaphthyl) maleimide.

The microbiocidal compounds useful in the practice of this invention which are isoindole dicarboximides having a sulfur atom bonded to the nitrogen atom of the dicarboximide group are compounds which contain at least one group having the structure:



The preferred isoindole dicarboximides are the following:



bis-N[(1, 1, 2, 2-tetrachloroethyl)thio]-4-cyclohexene-1, 2-dicarboximide,



n-trichloromethylthio-4-cyclohexene-1,2-dicarboximide,



N-trichloromethylthio phthalimide.

The halogenated aryl alkanols which can be used as microbiocidal compounds in accordance with this invention are exemplified by a preferred compound, 2,4-dichlorobenzyl alcohol.

An example of a preferred isothiazolinone compound useful in the composition of this invention is 2-(n-octyl-4-isothiazolin-3-one).

The most preferred microbiocidal compounds are the bisphenoxarsines and bisphenarsazines having the formula:



where Y is oxygen or sulfur and Z is oxygen or nitrogen. Of these bisphenoxarsines and bisphenarsazines, the most preferred are 10, 10'-oxybisphenoxarsine; 10, 10'-thiobisphenoxarsine; 10, 10'-oxybisphenarsazine; and 10, 10'-thiobisphenarsazine.

It is also within the scope of the invention to include other typical known antimicrobial agents such as bis(tri-n-butyl tin) oxide (TBTO) and the like.

Suitable media include those which are capable of dissolving or dispersing the antimicrobial agent. Obviously the selection of such medium is dependent on the nature of the agent such property would be readily determined by one skilled in the art. It is preferred that the medium be an aqueous liquid. It is also understood that various non aqueous constituents such as surfactants, leveling agents, buffers, dyes, organic solvents, etc. may be included in the media provided that such additional constituents do not interfere with the operation of the process.

The polyamides useful in this invention are conventional polymeric materials containing the amide linkage



5

and typified by solid polyamide polymers known generically as nylon. Included in the list of useful polyamides are those nylons designated as nylon 6, nylon 66, nylon 7, nylon 11 and others.

10 The polyamide material may be in any suitable solid form to facilitate efficient contact with the aqueous media containing the antimicrobial agent to be removed. Suitable solid forms may include granules, pellets, free-standing films, coatings on suitable substrates,

15 foams and fibers. Due to a favorable surface-to-volume ratio, fibers, or yarns and fabrics produced from polyamide fibers are preferred. However, the pellet form is also preferred due to ease of handling and other engineering consideration.

20 The invention may be practiced by simply contacting the antimicrobial agent containing aqueous media with a bed of polyamide material for sufficient time to allow all or a proportion of the agent to be absorbed by the polyamide absorbant. This contact method may be by

25 either batch or continuous processes. The efficiency of removal is governed by the proportion of antimicrobial agent present, relative to the quantity of polyamide material employed and the amount of aqueous media to be treated. The rate of removal is determined by factors that affect the attainment of equilibrium partitioning of the antimicrobial agent between the polyamide and aqueous phases. These factors include contact time, face velocity, temperatures, pH and surface area to volume ratio of the polymeric absorbant.

30 As an example of a batch technique for adjusting the antimicrobial agent concentration of aqueous media, one may periodically dip a porous holding container filled with polyamide material containing the agent in a concentration different than that of the media. On the

35 other hand, one could also continuously transfer and return the media from a treatment vessel, such as for example a beck dye bath, to another vessel containing a bed of the antimicrobial agent containing polyamide material. This procedure is illustrated in FIG. 1.

40 Other treatment vessels include conventional equipment utilized in dyeing of fibers. These are convenient vessels in which to hold the medium used for treatment of the fibers. For example, vats, stock dyeing, skein dyeing, rope dyers, continuous dye ranges, Kuesters or 45 Becks would be suitable.

A suitable apparatus system to conduct the process of the invention is illustrated in FIG. 1 in the form of a schematic diagram. Fiber 11 is passed through aqueous media 12 which is contained in treatment vessel 13.

50 Roller 20 is used to guide fiber 11 during its passage through vessel 13. The fiber is treated by the media to alter its antimicrobial agent content. The media may be passed intermittently or continuously into bed holding vessels 14 and 15 and then returned to vessel 13 through transfer pipes 16, 17, 18, and 19. Such passage is effected through use of pumps 21 and 22. Beds 23 and 24 are contained in vessels 14 and 15 and consist of polyamide materials which desirably have an antimicrobial agent concentration higher and lower, respectively, than that

55 of the media to be circulated through the beds. This would permit one to have the ability to raise or lower the concentration of the agent in the media wherever desired. Following treatment in treatment vessel 13,

fiber 11 may be passed through water rinse tank 25. The water from tank 25 may then be cleansed of carryover antimicrobial agent by connection with the treatment system by lines 26 and 27. Pumps 28 and 29 provide circulation for this portion of the system.

The following Examples serve to further illustrate the practice of the invention.

#### EXAMPLE I

##### Preparation of simulated beck dye bath

0.5 mL TRITON X-100 was added to 500 mL tap water. No pH adjustment was made. The pH was 6.8.

##### Treatment

The fiber and pellet weights and bath volumes used are shown in Table 1.

The simulated beck dye bath was heated to boiling in beakers covered with watch glasses. Untreated nylon fiber (yarn) samples were added to the bath simultaneously with nylon pellets containing 4.5% OBPA by HPLC suspended in nylon net bags. The solution containing both the fiber and pellets were heated together at 95° to 100° C. for 30 minutes. The samples were removed, squeezed, and rinsed in two 500 mL portions of deionized water at room temperature. The samples were squeezed and air dried.

#### EXAMPLE II

##### Simulated beck dye bath

1.0 mL Triton X-100 was added to 1 L tap water. No pH adjustment was made. The pH was 6.8.

##### Treatment—Timed Uptake

Fiber and pellet weights, bath volumes, and treatment times are shown in Table 1. Each fiber sample and pellet bag pair was added to individual beakers of boiling dye bath. At the appropriate time intervals the fiber and pellets were removed and rinsed in 1 L portions of deionized water and dried in a 45° oven overnight. 2 mL dye bath aliquots were removed, after fiber treatment, for arsenic analysis by SDDC.

##### Analyses of Treated Fibers

1-g samples of the treated fibers were soxhlet extracted overnight with methanol and analyzed for arsenic. The results are tabulated in Table 1. The results of the timed uptake experiment are shown graphically in FIGS. 2 and 3.

TABLE 1

| SAMPLE # | BATH TREATMENT OF NYLON FIBERS USING NYLON PELLETS CONTAINING OBPA |              |                          | OBPA FINAL BATH CONC. ppm | FIBER CONCENTRATION METHANOL EXTRACT, OBPA ppm | STAPH. ZONE SIZE mm |
|----------|--------------------------------------------------------------------|--------------|--------------------------|---------------------------|------------------------------------------------|---------------------|
|          | NYLON PELLETS WEIGHT GRAMS                                         | BATH Vol. mL | NYLON FIBER WEIGHT GRAMS |                           |                                                |                     |
|          | 4.5% OBPA                                                          |              |                          |                           |                                                |                     |
| 1        | 0.1384                                                             | 160          | 8.0535                   | 10                        | 1.7                                            | 18                  |
| 2        | 0.1459                                                             | 164          | 8.2022                   | 20                        | 2.4                                            | 36                  |
| 3        | 0.1432                                                             | 165          | 8.2582                   | 30                        | 3.3                                            | 70                  |
| 4        | 0.1463                                                             | 160          | 8.0908                   | 60                        | 4.2                                            | 125                 |
| CONTROL  | 0                                                                  | 80           | 4.3                      | 10                        | N.D.                                           | N.D.                |

I claim:

1. A method of adjusting antimicrobial agent concentration of an aqueous media, comprising:  
obtaining a first stream of antimicrobial agent containing aqueous media from an antimicrobial treatment vessel;  
passing said first stream through and in contact with a bed of solid polyamide absorbant material, said polyamide absorbant material containing a concentration of the same antimicrobial agent that is dif-

ferent from that in said first stream whereby the antimicrobial agent concentration in said stream is adjusted, said antimicrobial agent having a partition coefficient, defined as the ratio of antimicrobial agent absorbed by the polyamide absorbant relative to that retained in the aqueous media at equilibrium, of at least about 10:1 to either increase or decrease the antimicrobial concentration in said stream; and

- then returning said adjusted stream to said antimicrobial treatment vessel.
2. The method of claim 1 wherein:  
said antimicrobial agent is present in said bed of polyamide material in a concentration greater than that of said first stream whereby the antimicrobial agent concentration of said returned stream is higher than that of the first stream.
3. The method of claim 1, wherein:  
said antimicrobial agent is present in said bed of polyamide material in a concentration less than that of said first stream whereby the antimicrobial agent concentration of the returned stream is lower than that of the first stream.
4. The method of claim 1, wherein:  
said polyamide material comprises nylon.
5. The method of claim 4, wherein:  
said antimicrobial agent comprises 10,10'-oxybis-phenoxyarsine.
6. The method of claim 5, wherein:  
said nylon is in the form of a member selected from the group consisting of a fiber, a granule, a film, a foam, a coated article, and a pellet.
7. The method of claim 6, wherein:  
said nylon is in the form of a pellet.
8. The method of claim 1, wherein:  
said antimicrobial agent comprises 10,10'-oxybis-phenoxyarsine.
9. A system for adjusting antimicrobial agent concentration of an aqueous medium, comprising:  
a vessel for treating a fiber with an aqueous medium containing an antimicrobial agent, having a partition coefficient, defined as the ratio of antimicrobial agent absorbed by the polyamide absorbant relative to that retained in the aqueous media at equilibrium, of at least about 10:1 to either increase or decrease the antimicrobial concentration in said aqueous medium transfer means for passing and returning said medium from said treatment vessel to a second vessel which contains a bed of polyam-

ide absorbant material which contains the same antimicrobial agent as said aqueous medium, and transfer means for passing and returning said medium from said treatment vessel to a third vessel contains a bed of polyamide absorbant material which contains the same antimicrobial agent as said aqueous medium at a concentration less than said second vessel.

\* \* \* \* \*